

May 17, 1960

C. BARTELL ET AL

2,937,109

PRESSURE-SENSITIVE ADHESIVE TAPE

Filed May 7, 1956



INVENTORS

CHARLES BARTELL, CHARLES L.  
WEINER AND RICHARD M. SMITH  
BY

Morgan, Hauseman, Durden and Rine  
ATTORNEYS

# United States Patent Office

2,937,109

Patented May 17, 1960

1

2,937,109

## PRESSURE-SENSITIVE ADHESIVE TAPE

Charles Bartell, New Brunswick, Charles L. Weidner, Cranbury, and Richard M. Smith, Nixon, N.J., assignors, by mesne assignments, to Johnson & Johnson, New Brunswick, N.J., a corporation of New Jersey

Application May 7, 1956, Serial No. 583,198

3 Claims. (Cl. 117—122)

This invention relates to a normally tacky and pressure-sensitive adhesive sheet material and, more particularly, to a normally tacky and pressure-sensitive tape formed with a unified paper backing impregnated with a chloroprene polymer.

Paper-backed, normally tacky and pressure-sensitive adhesive tapes, particularly those used for masking purposes, should have high elongation, good flexibility, high edge tear, good tensile strength and adequate internal strength to prevent delamination of the backing upon unrolling of the tape. In the case of masking tapes, the product must have high elongation, flexibility and edge tear in order that the tape be curved to mask curved lines without tearing during application. The delamination resistance, or resistance of the backing to being split into two layers by forces perpendicular to the sheet, is necessary to enable unwinding of the tape and removal from the surface after it has served its intended function.

Paper backings for use in pressure-sensitive tapes can be unified or strengthened internally by treatment of the paper with aqueous latices of elastomeric polymers. The sheets are impregnated in amount sufficient to deposit substantial rubbery polymer solids in the web to bond the fibers thereof to a degree sufficient to lend the tape high internal strength. In the treatment of paper webs with latices, however, it has been generally found that the edge tear, elongation and flexibility of the sheet suffered considerably whenever ingredients were incorporated in the latex for the purpose of increasing the tensile strength and delamination resistance of the product. Obviously, a balancing of the characteristics of the tape is necessary to obtain a successful commercial product and increasing one property to the severe detriment of others is not advantageous. Another consideration is that the elastomeric polymer in unifying the paper must not cause a detrimental change in the appearance of the paper such as by effecting a discoloration thereof.

Accordingly, it is an object of this invention to provide a unified paper web suitable for use as a backing element for a normally tacky and pressure-sensitive adhesive sheet wherein the backing has the characteristics of high flexibility, elongation and edge tear and yet adequate tensile strength, and delamination resistance and wherein the appearance of the unified paper is not affected detrimentally.

It is an additional object of this invention to provide a normally tacky and pressure-sensitive paper tape having the aforementioned properties.

It is a further and more specific object of this invention to provide an impregnant composition for saturating paper webs to form backing elements with balanced properties of edge tear, flexibility, elongation, tensile strength and delamination resistance and wherein the appearance of the unified paper is not affected detrimentally.

It is a further object of this invention to provide a novel method for producing unified paper web and nor-

2

mally tacky and pressure-sensitive paper tape having the aforementioned characteristics.

These and other objects of the invention will become apparent when consideration is given to the hereinafter detailed description of the invention.

In accordance with this invention an open, porous saturable paper web is treated with an aqueous dispersion of a chloroprene polymeric elastomer to unify the paper in imparting satisfactory elongation, tensile strength and delamination resistance. It has been found that chloroprene polymeric elastomers are excellent unifying agents for this purpose. It has been further found, however, that such chloroprene polymers on aging cause a discoloration and embrittlement of the paper. While not being bound by any theory of action, the chloroprene polymer on aging appears to release HCl which attacks the paper tenderizing it and causing the paper to become brittle and crumbly. Moreover, the paper is discolored to an extent to render it commercially unattractive.

It has been found, however, that a chloroprene polymeric elastomer may be used successfully as a paper unifying agent if there is used in conjunction therewith a small amount of a compound which is a derivative of ammonia and commonly called an aminoacetic acid. The aminoacetic acids useful in accordance with this invention are derivatives of ammonia wherein at least one and preferably more than one of the hydrogens in ammonia is replaced by a group having the methyl carboxy radical, their salts and ethers. One hydrogen may also be replaced by an alkyl amine or by a compound having an alkyl amine methyl carboxy radical and preferably having two methyl carboxy radicals. Also, one or more hydrogens may be replaced by ethyloxy groups. Thus the simplest compound within this group is aminoacetic acid [ $\text{NH}_2\text{CH}_2\text{COOH}$ ] and more complex compounds are aminodiacetic acid [ $\text{NH}(\text{CH}_2\text{COOH})_2$ ], diethyloxy aminoacetic acid [ $\text{N}(\text{CH}_2\text{CH}_2\text{OH})_2\text{CH}_2\text{COOH}$ ], amino triacetic acid [ $\text{N}(\text{CH}_2\text{COOH})_3$ ], ethylene diamine diacetic acid [ $\text{C}_2\text{H}_4(\text{NHCH}_2\text{COOH})_2$ ] and related compounds such as ethylene diamine tetraacetic acid [ $\text{C}_2\text{H}_4\text{N}_2(\text{CH}_2\text{COOH})_4$ ], and ethylene diamine (ethyloxy) triacetic acid [ $\text{C}_2\text{H}_4\text{N}_2(\text{CH}_2\text{CH}_2\text{OH})(\text{CH}_2\text{COOH})_3$ ]. The alkyl chains in these compounds may be materially longer than in the last mentioned case, as for instance, in the case of butylenediamine di-acetic acid



Instead of acids their salts and esters may be used, for instance the mono-N-butyl amine salt of ethylene diamine tetraacetic acid



It appears that the location within the molecule and size of the alkyl chains in these compounds is not of great importance as far as their protective properties are concerned and that satisfactory results may be obtained by using any compounds having any desired number of carboxyl radicals, including particularly acids, amine salts and also salts based on mono-valent alkali metals, i.e. sodium, potassium and lithium. In addition, water soluble monovalent salts such as mono calcium, mono lead and mono zinc salts may be used.

Among preferred materials with this group are any of the amine salts of the ethylene diamine polyacetic acids such as the diethyl amine salts and the butyl amine salts, and the univalent alkali metal salts of these acids, such as the sodium, potassium and lithium salts. In like manner esters of the acids may also be used. The alkyl and alkylene chains in the molecules may be short as in the case of the ethyl esters and ethyl amine salts or quite long as in the case of the octyl and diethylene esters and octyl amine salts. Chains of intermediate

length also serve satisfactorily. Di-, tri-, or tetra-acetates may be used in this invention and nitrilotriacetic acid and its esters and salts are well suited for its purposes. The preferred amino acetates cause little or no stains on materials which they contact.

The preferred compounds to be used as protective agents with chloroprene polymers may be expressed by the formula



wherein  $R_1$  is selected from the group consisting of  $-H$ ,  $-CH_2CH_2OH$ ,  $-CH_2COO-D+$ , and



wherein  $R_2$  and  $R_3$  each are selected from the group consisting of  $-H$ ,  $-CH_2CH_2OH$ ,  $-CH_2COO-D+$ , and  $-CH_2COOR_4$  wherein  $R_4$  is an alkyl radical having from two to five carbon atoms in the chain; wherein  $D$  is a cation selected from the group consisting of  $H^+$ ,  $Na^+$ ,  $K^+$ ,  $Li^+$ ,  $NH_4^+$ , and  $NA_3H^+$ ; wherein  $A$  is at least one of the members of the group consisting of hydrogen, alkyl and ethanol; and wherein  $x$  is at least 2 and not more than 4.

It has been found that papers impregnated with a composition containing a chloroprene polymer and an amino-acetic acid of the aforementioned type exhibit satisfactory flexibility, tensile strength, elongation and delamination resistance for use as a backing for paper tapes. Unified papers, produced in this manner, will not become discolored or brittle on aging in contrast to paper unified with chloroprene polymers in the absence of the amino-acetic acid. Unified papers formed in accordance with this invention can be applied in sharp curve fashion without tearing. Consequently, when used as a masking tape, the line of demarcation of paint is continuously smooth so that no refinishing operations of the painted surfaces are required. Moreover, the masking tapes of this invention are of a high flexibility, so that they adhere to uneven or curved surfaces without difficulty. They exhibit no tendency to lift or curl easily, remaining strongly adhered to the surfaces to which they are applied so that there is no opportunity for paint to seep underneath the tape to destroy the purpose of said masking tape.

The exact mechanism of the aminoacetic acid in preventing discoloration of the paper by aging of the chloroprene polymer impregnant is not known. It does not function as a mere acid acceptor, however, for  $ZnO$  a commonly used acid acceptor gives an overall protec-

sheet material of this invention, so long as the web is porous and can be completely saturated. The web may be made in part or in whole from wood, rope or rag fibers or other fibrous material, natural or synthetic.

5 Preferably, paper webs of the conventional type employed as backings for normally tacky and pressure-sensitive adhesive tapes, such as those formed of kraft pulp and the like, are used. The paper may be flat or it may be creped, crimped, embossed or otherwise treated so as to provide rugosities or corrugations whereby stretchability of the sheet is increased.

10 The preparation of polychloroprene from chloroprene is well known. After suitable purification by careful fractionation, chloroprene is emulsified in water by means of sodium rosinate soap and polymerized at 40° C. with the aid of potassium persulfate as a catalyst, and in the presence of elemental sulfur as a modifier. A basic polymerization recipe is as follows:

|                                                   | Parts   |
|---------------------------------------------------|---------|
| 20 Chloroprene                                    | 100     |
| N wood rosin <sup>1</sup>                         | 4       |
| Sulfur <sup>1</sup>                               | 0.6     |
| Water                                             | 150     |
| Sodium hydroxide                                  | 0.8     |
| 25 Sodium salt of naphthalene-sulfonic acid-form- |         |
| aldehyde condensation product                     | 0.7     |
| Potassium persulfate                              | 0.2-1.0 |

<sup>1</sup> Dissolved in monomer.

30 Moreover, chloroprene can be copolymerized with relatively small amounts of other monomers. For example, styrene comonomer tends to make a polychloroprene with less crystallization tendencies, isoprene comonomer tends to make for better low-temperature service, and acrylonitrile for good processibility and oil resistance.

35 Examples of suitable chloroprene (2-chloro-butadiene) polymers useful in accordance with this invention are the neoprene rubbers. Neoprene is a generic name applied to polymers of chloroprene or mixtures of chloroprene and other polymerizable monomers; the major constituent of which is chloroprene.

40 Specific examples of neoprene latices are those manufactured by the Du Pont Company, Wilmington, Delaware, and sold under the trade names of "Neoprene 571," "Neoprene-842-A," "Neoprene 601-A," "Neoprene 735" and "Neoprene 572." All of these latices are alkaline dispersions of polymerized chloroprene (2-chloro-1,3-butadiene) in water containing dispersing and stabilizing agents. Specific data for these latices are shown in the following Table I:

TABLE I

| Chloroprene Polymer | Solids, Percent By Weight | Specific Gravity | Initial pH | Average Limiting Viscosity, cps. | Surface Tension, Dynes/cm. | Emulsifying Agent                      | Particle Diameter, Microns |
|---------------------|---------------------------|------------------|------------|----------------------------------|----------------------------|----------------------------------------|----------------------------|
| Neoprene 571        | 50                        | 1.10             | 12.1       | 8.0                              | 36                         | Sodium Rosinate                        | 0.13                       |
| Neoprene 842-A      | 50                        | 1.10             | 12.4       | 8.0                              | 36                         | do                                     | 0.13                       |
| Neoprene 601-A      | 59                        | 1.12             | 12.2       | 35.0                             | 42                         | do                                     | 0.13                       |
| Neoprene 735        | 36                        | 1.08             | 12.2       | 6.0                              | 36                         | Sodium Salt of Disproportionated Rosin | 0.11                       |
| Neoprene 572        | 60                        | 1.10             | 12.2       | 8.0                              | 36                         | Sodium Rosinate                        | 0.13                       |

tive action against discoloration far interior to that obtained by using an amino-acetic acid. In like manner, the aminoacetic acid does not function as a mere antioxidant, for the protective action effected by it is far superior to that obtained by using "Agerite White" (di-B-naphthyl-p-phenylene diamine), a commonly used antioxidant for neoprene rubber products or 2,2, methylene bis (4 methyl-6-tert-butyl phenol), another commonly recommended neoprene antioxidant.

Various types of fibrous webs may be employed as the

70 In accordance with this invention, the fibrous web is impregnated with a chloroprene latex in amount sufficient to enable incorporation of the dry solids of the impregnant into the sheet in amount approximately 20 to 150%, and preferably 65 to 100% by weight of the dry non-impregnated sheet. In general, the aminoacetic acid is in an amount from about 0.2 to about 10% by weight of the chloroprene polymer. Amounts less than the indicated minimum range (0.2%) do not always exert the desired protective action against discolor-

oration while amounts greater than 10% tend to destabilize the latex. After impregnation, the saturated webs are dried at a suitable temperature as for example 100-250° F. Of course, it will be appreciated that a lower temperature of drying requires a longer time for drying.

The novel and unusual features of this invention can best be shown by the following examples. It will be noted that Examples III, VI, VIII and X are examples of latices prepared in accordance with this invention while the latices disclosed in the remaining examples are disclosed for the purpose of comparison to highlight the novel features of the present invention. It should be noted that two temperatures, 200° and 250° F., were used for accelerated aging; 16 hours at 200° F. is a mild aging condition, 65 hours is a moderate aging condition, whereas 182 hours at 200° F. or 16 hours at 250° F. is a severe aging condition.

#### Example I

This example illustrates the production of a unified paper employing a chloroprene latex but containing no aminoacetic acid protective agent.

A 38-pound creped saturating paper was saturated with an equal dry weight of polychloroprene latex (Neoprene 735) having a Mooney viscosity of 68. The impregnation was accomplished with conventional squeeze roll equipment and the wet sheet dried in an air circulating oven at 250° F. The freshly impregnated sheet was light tan in color. When the same sheet was heat aged in an air circulating oven for merely 16 hours at 200° F. it turned dark brown and the paper was so brittle it tended to crumble. When heated 16 hours at 250° F., the paper turned brown-black and just crumbled.

#### Example II

This example illustrates the production of a unified paper utilizing a latex comprising chloroprene and a commonly used acid acceptor, namely, zinc oxide. A 27 pound creped saturating paper was saturated with 85% of its weight (dry basis) of a latex composition consisting of 90% polychloroprene (Mooney=60) and 10% of a dispersed zinc oxide. The freshly impregnated sheet was of a very light tan color and flexible. When heat aged for 65 hours at 200° F. it turned medium brown in color, became somewhat brittle. When heated 16 hours at 250° F. it turned dark brown in color, tended to crumble.

#### Example III

This example illustrates the preparation of a unified paper in accordance with the invention utilizing a latex comprising polychloroprene and an aminoacetic acid (sodium salt of ethylene diamine-tetra-acetic acid) as a protective agent. A 30 lb. flat kraft paper was saturated with 75% of its weight (dry basis) of a latex composition consisting of 97% polychloroprene (Mooney=60) and 3% of the sodium salt of ethylene diamine-tetra-acetic acid. The freshly impregnated sheet was light tan in color and flexible. When aged 182 hours at 200° F. the paper was still light in color and flexible. When aged 16 hours at 250° F. no significant change in color was noted and the paper remained flexible.

#### Example IV

This example illustrates the production of a unified paper utilizing a latex comprising polychloroprene and a commonly used neoprene antioxidant, namely 2,2-methylene bis (4-methyl-6-tert-butylphenol).

A 4-mil rope paper was saturated with 50% of its weight (dry basis) with a latex composition consisting of 97% polychloroprene (Mooney=45) and 3% 2,2-methylene bis (4-methyl-6-tert-butylphenol). The fresh-

ly impregnated sheet was light tan in color and flexible. When aged 65 hours at 200° F. it turned slightly darker and was still flexible. When aged 182 hours at 200° F. for 16 hours at 250° F., it turned dark brown, became brittle and crumbly.

#### Example V

This example illustrates the production of a unified paper utilizing a latex comprising polychloroprene, a commonly used acid acceptor ZnO and a commonly used neoprene antioxidant 2,2-methylene bis (4-methyl-6-tert-butylphenol).

A 4-mil rope paper was saturated with 75% of its weight (dry basis) with a latex composition consisting of 87% polychloroprene (Mooney=45), 10% dispersed zinc oxide and 3% 2,2-methylene bis (4-methyl-6-tert-butylphenol). The freshly impregnated sheet was very light tan in color and flexible. When aged 182 hours at 200° F. or 16 hours at 250° F. it turned dark brown in color and became stiff.

#### Example VI

This example illustrates the production of a unified paper in accordance with this invention utilizing a latex comprising a polychloroprene, an aminoacetic acid (sodium salt of ethylene diamine-tetra-acetic acid) and an antioxidant 2,2-methylene-bis (4-methyl-6-tert-butylphenol).

A 4-mil rope saturating paper was saturated with 50% of its weight (dry basis) with a latex composition consisting of 95% polychloroprene (Mooney=45), 3% 2,2-methylene-bis (4-methyl-6-tert-butylphenol) and 3% sodium salt of ethylene diamine tetraacetic acid. The freshly impregnated sheet was light in color and flexible. When aged 182 hours at 200° F. or 16 hours at 250° F. it turned light brown in color, but was considerably lighter in color than that of Example IV which used the antioxidant alone, and was lighter than that of Example V which used both an antioxidant and acid acceptor. The paper remained flexible.

#### Example VII

The same as in Example V except that di-beta-naphyl-paraphenylene diamine was used as the antioxidant in place of 2,2-methylene-bis-(4-methyl-6-tert-butyl-phenol). The freshly prepared sheet was light in color. After a week of natural aging it turned pink in color. Upon heat aging 65 hours at 200° F. it turned grey green and after 15 hours at 250° F. it turned dark grey. The paper remained flexible.

#### Example VIII

This is another example of a sheet unified in accordance with this invention. This example is the same as in Example VI except that di-beta-naphyl paraphenylene diamine was used in place of 2,2-methylene-bis (4-methyl-6-tert-butyl-phenol). Again as in Example VII on naturally aging the paper tended to turn pink. However, on heat aging, the samples remained lighter than those of Example VII.

#### Example IX

The same as in Example IV except that the antioxidant used was hydroquinone monobenzyl ether in place of 2,2-methylene-bis (4-methyl-6-tert-butylphenol). The freshly impregnated sheet was light tan in color but became brown under aging conditions of 65 hours at 200° F.

#### Example X

This is another example in accordance with the invention and is the same as in Example VI except that hydroquinone monobenzyl ether is used in place of 2,2-methylene-bis (4-methyl-6-tert-butyl-phenol). Upon heat

aging 65 hours at 200° F., the unified paper was lighter in color than that of Example IX.

Examples of additional unified papers prepared in accordance with the present invention are as follows:

*Example XI*

A 27-pound creped saturating paper was saturated with 85% of its weight (dry basis) of a latex composition consisting of 98% polychloroprene (Mooney=60) and 2% of the trisodium salt of ethylene diamine ethylole triacetic acid— $[C_2H_4N_2(CH_2CH_2OH)](CH_2COONa)_3$ .

*Example XII*

A 70-pound flat kraft paper was saturated with 25% of its weight (dry basis) of a latex composition consisting of 99% polychloroprene (Mooney=45) and 1% of the pentasodium salt of N,N,di(ethylamine diacetic acid) glycine— $[C_2H_4(CH_2COONa)_2]_2NCH_2COONa$ .

*Example XIII*

A 4-mil rope saturating paper was saturated with 100% of its weight (dry basis) with a latex composition consisting of 88% polychloroprene (Mooney=45), 10% of the disodium lead salt of ethylene diamine tetraacetic acid— $(CH_2COO)_2Pb(C_2H_4N_2)(CH_2COONa)_2$  and 2% of a non-ionic salt such as "Triton X-100" sold by Rohm & Haas, Philadelphia, Pennsylvania, the salt being necessary to stabilize the latex prior to addition of the antioxidant. The freshly impregnated sheet was light in color. When aged 16 hours at 250° F., the sheet remained light in color and flexible.

As indicated heretofore, the unified papers formed in accordance with this invention are particularly useful as backings of normally tacky and pressure-sensitive tapes. Any suitable normally tacky and pressure-sensitive adhesive useful in paper tapes may be used. Such adhesives are generally compounded from a composition of synthetic rubber or similar elastomeric polymer, and a resinous component compatible with the rubber and adapted to impart tack to the adhesive composition, together with suitable amounts of various types of additives such as conventional fillers, antioxidants, etc. The elastomeric component, tackifying resin, and fillers, when used, are proportioned to obtain in the adhesive properties of high internal strength and cohesiveness and high adhesiveness. As shown in the figure in cross-section, the adhesive tape comprises a unified backing having coated on one side a suitable normally tacky and pressure-sensitive adhesive.

Examples of specific adhesive compositions useful in forming the novel tapes in accordance with this invention are as follows:

**TYPE A**

|                                       |     |
|---------------------------------------|-----|
| Milled pale crepe rubber              | 100 |
| Polybetapinene resin                  | 75  |
| Petroleum oil                         | 5   |
| Polymerized trimethyldihydroquinoline | 2   |

**TYPE B**

|                                             |     |
|---------------------------------------------|-----|
| Milled smoked sheet rubber                  | 100 |
| Zinc oxide                                  | 50  |
| Dehydrogenated rosin                        | 75  |
| Sym. di-beta-naphthyl-paraphenylene diamine | 2   |
| Lanolin                                     | 10  |

**TYPE C**

|                                                                             |    |
|-----------------------------------------------------------------------------|----|
| Butadiene-styrene copolymer (butadiene-styrene ratio 70:30 Mooney value 50) | 50 |
| Smoked sheet                                                                | 50 |
| Ester of hydrogenated rosin                                                 | 50 |
| Polymerized trimethyldihydroquinoline                                       | 2  |
| Petroleum oil                                                               | 20 |

**TYPE D**

|                                                 |      |      |
|-------------------------------------------------|------|------|
| Polyvinyl ethyl ether resin intrinsic viscosity | 2.37 | 100  |
| Hydrogenated rosin                              |      | 5    |
| Phenylalpha naphthylamine                       |      | 0.35 |
| 5 Polyethylene glycol 400 (di, tri) ricinoleate |      | 1.5  |

**TYPE E**

|                                         |     |
|-----------------------------------------|-----|
| Polyisobutylene high polymer, solid     | 100 |
| Polyisobutylene polymer, viscous liquid | 70  |
| 10 Toluene                              | 520 |

In forming the novel paper tapes of this invention, the adhesive may be applied to the unified paper of the invention in any conventional manner, as for example 15 by calendering, reverse roll-coater, knife-coater, etc. The adhesives are preferably applied to the unified paper from solvent solution or dispersion using aliphatic or aromatic solvents and subsequent drying. If desired, the backing may be provided with a suitable conventional 20 priming coating to improve the adherence of the coating thereto.

Preferably, the paper tapes of this invention are provided with a backsize composition on the side opposite the adhesively coated side of the unified backing. Also, 25 if desired a release coating may be applied over the backsize coating, the backsize acting as a base coat in anchoring the release coating to the backing. The use of a release coating is particularly desirable wherein the delamination resistance is not as high as desired. Examples 30 of suitable backsize composition for the above purpose are nitrocellulose, vinyl chloride-acetate copolymers and similar film formers.

The following is an example for the preparation of a 35 normally tacky and pressure-sensitive adhesive tape in accordance with the present invention:

*Example XIV*

A normally tacky and pressure-sensitive tape is produced by coating in a conventional manner the chloroprene-sodium salt of ethylene diamine tetraacetic acid impregnated flat kraft paper of Example III with the pale crepe rubber adhesive Type A at a coating weight of about 1.5 ounces per sq. yd. of paper, drying the adhesive coating, and coating the opposite side of the paper with 0.3 ounce per square yard of a nitrocellulose backsize composition.

The invention in its broader aspects is not limited to the specific steps, compositions, combinations and improvements shown and described but departures may be made therefrom within the scope of the accompanying claims without departing from the principles of the invention and without sacrificing its chief advantages.

What is claimed is:

55 1. A paper-backed normally tacky and pressure-sensitive adhesive tape having satisfactory flexibility, elongation, edge tear resistance, delamination resistance and resistance to discoloration comprising a unified paper sheet 40 comprising a fibrous web internally bonded with a composition comprising a major amount of bonding particles 45 including a chloroprene polymer and about 0.2 to 10% by weight of the chloroprene polymer of an aminoacetic acid compound of the formula



70 wherein  $R_1$  is selected from the group consisting of  $—H$ ,  $—CH_2CH_2OH$ ,  $—CH_2COO—D+$ , and  $—(CH_2)_xNR_3$ ,  $CH_2COO—D+$  wherein  $R_2$  and  $R_3$  each are selected 75 from the group consisting of  $—H$ ,  $—CH_2CH_2OH$ ,  $—CH_2COO—D+$ , and  $—CH_2COOR_4$  wherein  $R_4$  is an

alkyl radical having from two to five carbon atoms in the chain; wherein D is a cation selected from the group consisting of H<sup>+</sup>, Na<sup>+</sup>, K<sup>+</sup>, Li<sup>+</sup>, NH<sub>4</sub><sup>+</sup>, and Na<sub>3</sub>H<sup>+</sup>, wherein A is at least one of the members of the group consisting of hydrogen, alkyl and ethylool and wherein x is at least 2 and not more than 4, said web having at least one major surface thereof coated with a normally tacky and pressure-sensitive adhesive.

2. A paper-backed normally tacky and pressure-sensitive adhesive tape in accordance with claim 1 wherein the chloroprene polymer is in an amount of 20 to 150% by weight of the fibrous web.

3. A paper-backed normally tacky and pressure-sensitive adhesive tape in accordance with claim 1 wherein the aminoacetic acid compound is the sodium salt of ethylene diamine tetraacetic acid.

## References Cited in the file of this patent

## UNITED STATES PATENTS

|           |            |               |
|-----------|------------|---------------|
| 2,287,063 | Raynolds   | June 23, 1942 |
| 2,442,972 | Edelstein  | June 8, 1948  |
| 2,485,458 | Quinn      | Oct. 18, 1949 |
| 2,492,702 | Neubert    | Dec. 27, 1949 |
| 2,560,743 | Rhenes     | July 17, 1951 |
| 2,697,700 | Uraneck    | Dec. 21, 1954 |
| 2,751,365 | Scott      | June 19, 1956 |
| 2,754,291 | Pollack    | July 10, 1956 |
| 2,765,228 | Jordan     | Oct. 2, 1956  |
| 2,765,229 | McLaughlin | Oct. 2, 1956  |

## FOREIGN PATENTS

|         |               |              |
|---------|---------------|--------------|
| 551,113 | Great Britain | Feb. 8, 1943 |
|---------|---------------|--------------|

UNITED STATES PATENT OFFICE  
CERTIFICATE OF CORRECTION

Patent No. 2,937,109

May 17, 1960

Charles Bartell et al.

It is hereby certified that error appears in the printed specification of the above numbered patent requiring correction and that the said Letters Patent should read as corrected below.

Column 3, line 66, for "interior" read -- inferior --; column 7, line 20, the formula should appear as shown below instead of as in the patent:



Signed and sealed this 4th day of April 1961.

(SEAL)

Attest: ERNEST W. SWIDER

XXXXXX  
Attesting Officer

ARTHUR W. CROCKER  
Acting Commissioner of Patents